

## UNITED STATES PATENT OFFICE

2,185,996

## HIGH TENSILE ALLOY STEEL

William Herbert Hatfield, Sheffield, England, assignor to Thos. Firth & John Brown Limited, Sheffield, Yorkshire, England, a British company

No. Drawing. Application December 10, 1937,  
Serial No. 179,123. In Great Britain February  
5, 1937

2 Claims. (Cl. 75—128)

This invention consists in a new or improved high tensile alloy steel.

In order to obtain steels of high tensile strength for structural purposes and other high duty applications, it has been general practice to employ the addition of certain elements to the composition, which in conjunction with the carbon content rendered the steel capable of being hardened and tempered, the latter operation giving a degree of control over the residual hardness and tensile strength in conjunction with the elimination of brittleness generally left as a result of the hardening operation.

The present invention relates to a new combination of iron and alloying elements which contains no great amount of carbon, and gives a substantially high tensile strength in combination with a high degree of ductility. This combination has the advantages that over a wide range of tempering temperatures its hardness and tensile strength fall comparatively slowly, thus giving a distinct advantage in heat treatment operation.

The invention provides an alloy steel of the type containing small proportions of nickel and chromium (say up to 7% of each element) together with molybdenum, characterised in that the carbon content does not exceed 0.12%, while the molybdenum content is relatively high for this type of steel, namely of the order of 2 to 5%.

More specifically, the invention consists in an alloy steel having the following composition:

|            | Per cent  |
|------------|-----------|
| Carbon     | 0 to 0.12 |
| Nickel     | 3 to 7    |
| Chromium   | 3 to 7    |
| Molybdenum | 2 to 5    |

with or without the usual percentages of other elements such as silicon and manganese, employed in steel making operations. It is, however, within the scope of the invention to add somewhat higher proportions of manganese in quantities up to say 5%, as this element tends to produce the desired properties. If desired, tungsten may be added in quantities not exceeding 4 or 5%.

A typical example of such a steel in accordance with the invention and with the mechanical properties obtained is as follows:

| Analysis Percent |      |   |  |  |  |  |  |  |  |
|------------------|------|---|--|--|--|--|--|--|--|
| Carbon           | 0.08 |   |  |  |  |  |  |  |  |
| Silicon          | 0.54 |   |  |  |  |  |  |  |  |
| Manganese        | 0.54 | 5 |  |  |  |  |  |  |  |
| Nickel           | 5.00 |   |  |  |  |  |  |  |  |
| Chromium         | 4.16 |   |  |  |  |  |  |  |  |
| Molybdenum       | 3.18 |   |  |  |  |  |  |  |  |

| Hardness tests.<br>(30 kg. Brinell) | As<br>forged | 10   |      |      |      |      |      |      |       |    |
|-------------------------------------|--------------|------|------|------|------|------|------|------|-------|----|
|                                     |              | 650° | 700° | 750° | 800° | 850° | 900° | 950° | 1000° |    |
| Air cooled                          | —            | 333  | 366  | 393  | 398  | 398  | 398  | —    | 351   |    |
| Oil quenched                        | —            | 320  | 321  | 360  | 377  | 393  | 398  | 377  | 364   |    |
| Water quenched                      | 387          | 329  | 321  | 360  | 386  | 375  | 388  | 388  | 375   | 15 |

| MECHANICAL PROPERTIES                                 |  |  |  |  |  |  |  |  |  |
|-------------------------------------------------------|--|--|--|--|--|--|--|--|--|
| (Tests on 0.423" x 1½"). Treated as 7/8" diameter bar |  |  |  |  |  |  |  |  |  |

|                   | Treatment: Air cooled from 900° C.—air cooled after tempering for 1 hour at— |            |            |            |
|-------------------|------------------------------------------------------------------------------|------------|------------|------------|
|                   | 200° C.                                                                      | 500° C.    | 600° C.    |            |
| Yield point       | tons/sq. in.                                                                 | 71.8       | 80.4       | 53.8       |
| Maximum stress    | tons/sq. in.                                                                 | 85.5       | 87.8       | 70.6       |
| Elongation        | percent                                                                      | 18.4       | 20.8       | 26.4       |
| Reduction of area | percent                                                                      | 53.0       | 56.0       | 62.0       |
| Izod test         |                                                                              | 38, 36, 34 | 37, 40, 37 | 57, 54, 56 |

|                   | Treatment: Oil quenched from 900° C.—air cooled after tempering for 1 hour at— |            |            |            |
|-------------------|--------------------------------------------------------------------------------|------------|------------|------------|
|                   | 200° C.                                                                        | 500° C.    | 600° C.    |            |
| Yield point       | tons/sq. in.                                                                   | 79.0       | 76.9       | 52.2       |
| Maximum stress    | tons/sq. in.                                                                   | 85.7       | 86.0       | 69.0       |
| Elongation        | percent                                                                        | 20.0       | 22.4       | 26.4       |
| Reduction of area | percent                                                                        | 55.0       | 61.0       | 65.5       |
| Izod test         |                                                                                | 37, 35, 37 | 39, 40, 42 | 56, 64, 62 |

I claim:

1. A high tensile alloy steel containing about 5% nickel, 4% chromium, 3% molybdenum, 0.08% carbon, 0.5% silicon, 0.5% manganese, and the remainder iron, the alloy being quenched from about 900° C. and subsequently tempered and air cooled from the tempering temperature. 45  
50

2. A high tensile alloy steel containing nickel above 3% and up to 7%, chromium 3-7%, molybdenum above 2% and up to 5%, carbon a trace up to a maximum of 0.12% and the remainder being substantially all iron except incidental impurities, the alloy being air cooled from about 900° C. and subsequently tempered for 1 hour and air cooled from the tempering temperature,

and the alloy having the following mechanical properties for the tempering temperatures given:

| Tempering temperature              | 200° C. | 500° C. | 600° C. |
|------------------------------------|---------|---------|---------|
| Yield point tons/sq. in. at least  | 71      | 80      | 53      |
| Elongation percent at least        | 18      | 20      | 26      |
| Reduction in area percent at least | 53      | 56      | 62      |

WILLIAM HERBERT HATFIELD.